

3,408,710

## PROCESS FOR THE MANUFACTURE OF BERYLLIUM PRODUCTS

José Mallen-Herrero, Paris, and Michel Weisz, Orsay, France, assignors to Commissariat à l'Energie Atomique, Paris, France

No Drawing. Filed Oct. 19, 1964, Ser. No. 404,906

Claims priority, application France, Oct. 25, 1963,

951,894

3 Claims. (Cl. 29—423)

### ABSTRACT OF THE DISCLOSURE

A cast beryllium ingot is covered with a thin soft steel coating; compressed at 800° C.; extruded at about 900° C.; covered with a thick soft steel envelope; and forged. After heating to 1000° C. the ingot is compressed and the steel cover removed. The billet may be coated with silver and then extruded at 900° C.

The present invention relates to improvements in processes for the manufacture of beryllium products as used particularly in the fields of aviation, aeronautics and atomic energy.

The invention is concerned more particularly with processes for the manufacture of beryllium tubes, and more particularly tubes suitable for casing the fuel elements of nuclear reactors.

Since the beginning of the use of beryllium in aircraft, and then for spacecraft, and finally as a nuclear material, for which fields it is particularly suitable by virtue of its remarkable properties, the desired beryllium products have been produced from billets or blooms of sintered beryllium. Only some parts of simple shape, such as sheets, have been obtainable from cast metal, and in addition it has been necessary to proceed with a grain refinement in order that this material may have acceptable mechanical characteristics.

In the past attempts have been made to improve the ductility of beryllium tubes and for this reason recourse has been had to powder metallurgy for the manufacture of such tubes, the sintered metal having a much finer grain than the cast metal, and also much higher longitudinal ductility, at ambient temperature.

The present invention relates to a process for the preparation of beryllium products and particularly tubes, which more fully satisfies than hitherto the various practical requirements, notably by virtue of the fact that it makes it possible to obtain a less fragile product of more favourable texture in the sense that it conforms to the following two characteristics:

(1) The base planes of the elemental crystallites are for the greater part disposed in parallel relationship to the extruding direction,

(2) The maximum angular distribution of these planes is located in the tangential direction.

For this purpose, the process according to the invention consists mainly—while using a cast beryllium ingot as starting material, optically subjected to compression—in subjecting it, in the course of its shaping, to at least one hot working operation followed by a forging, notably in a press, optionally under a thick steel casing, and by at least one further extrusion performed after removal of the casing, when necessary.

Apart from this main feature, the invention further comprises other features which are preferably used at the same time, considered separately or in all the technical possible combinations:

(a) The said hot working operation consists in an extrusion in a casing, which casing may consist of soft steel, and

(b) The second extrusion consists in an impact extrusion, the metal being coated with a thin layer of silver.

In any case, it will be more readily understood from the following further description and from the following examples, which further description and examples are, of course, given only by way of example and have no limiting character.

The use of cast metal as starting material, instead of sintered metal as is usual, is a feature of the present invention, because it is found that hot worked cast metal is substantially free from hot fragility, that its texture is more favourable than that of hot worked sintered metal, that the maintenance at a temperature of 600° or 700° C. for long periods is beneficial to hot worked cast metal, while being harmful to hot worked sintered metal, that radiographs of inclusions have revealed higher "cleanliness" of the hot worked metal, and finally that, although its presentation and its surface appearance do not appear to be so good, it is less subject to defects such as intergranular microcracks, which are harmful to transverse ductility in the case of tubes.

The following table shows a comparison of the longitudinal and transverse ductilities in the case of ingots of sintered and cast beryllium.

|                             | Minimum temperature for an elongation of 10% |               |
|-----------------------------|----------------------------------------------|---------------|
|                             | Longitudinal                                 | Transverse    |
| Extruded sintered sheet bar | 50° C.                                       | Above 400° C. |
| Extruded cast sheet bar     | 140° C.                                      | 250° C.       |

Since the transverse ductility is much greater than the longitudinal ductility in the case of tubes, notably for casings, the superiority of cast beryllium will be seen from this table.

After the choice of the cast metal, the choice of the hot working operation acts as a second factor. Methods as different as impact extrusion and the conventional cased extrusion technique may be employed, this second method, however, giving tubes of greater length and greater homogeneity.

It is found that a further means of improving the transverse ductility  $D_T$  is to vary the angular distribution of the base planes. If these are radially disposed (as in the case of a tube), longitudinal fissures will tend to appear and cleavage will be facilitated.

Attempts have been made to produce tubes having a texture characterised by the following points:

(1) The base planes of the elemental crystallites disposed for the greater part in parallel relationship to the extruding direction, and

(2) Maximum angular distribution of these planes in the tangential direction.

There will therefore be given in the following an example of the production of beryllium tubes by the process according to the present invention.

#### Example

A cast metal cylinder is coated with a thin layer of soft steel 2 mm. thick. The whole is compressed at 800° C., and then extruded at about 900° C. with a cold working degree of 6. A bar 40 mm. in diameter is obtained, from which a billet is sliced.

This billet is disposed in a soft-steel envelope 10 mm. thick and will be subjected to the forging operation. After heating to about 1000° C., the billet together with its envelope is compressed in the press along its axis so as to bring its height from the value  $H$  to the value  $h$ .

The extent of deformation thus obtained is:

$$\frac{H-h}{H} = 0.25$$

The billet time thus deformed is thereafter freed from its steel envelope, machined, drilled and coated with a thin silver layer.

Impact extrusion is then effected at about 900° C. to a hot working degree of 15. The tubes thus obtained have an external diameter of 15.2 mm. and an internal diameter of 13.2 mm.

They exhibit a distribution of the orientations of the base planes (0002) having a very pronounced maximum in the tangential direction, and a minimum in the radial direction, the maximum/minimum ratio being equal to about 6, thus illustrating the marked predominance of the tangentially disposed planes. In the particular application to the casing of fuel elements in gas-cooled nuclear reactors, it therefore appears that the probability of breakage and consequent liberation of the fission products in the cooling gas will be greatly reduced by the use of beryllium tubes produced by the process of the present invention, which gives a tangential disposition of the base planes of the elemental crystallites.

Of course, the invention is in no way limited to the mode of application which has just been referred to, nor to the embodiment described by way of example, but covers all variants thereof, and notably the production of beryllium products from cast metal, not only for nuclear uses, but also for the requirements of aviation and aeronautics.

#### What we claim is:

1. In a process for the manufacture of beryllium products, the steps of coating an ingot of cast beryllium with

a thin layer of soft steel, then subjecting said coated ingot to compression at about 800° C., then subjecting said ingot in the course of shaping to at least one hot working operation at about 900° C., then applying a thick steel casing to said ingot, then forging said ingot at about 1000° C. in a press, then removing said thick casing and then subjecting said ingot to at least one further hot working.

5 2. A process as described in claim 1, said hot working operation comprising an extrusion under a soft steel casing.

10 3. A process as described in claim 1, said second extrusion comprising an impact extrusion, said ingot being coated with a thin layer of silver.

#### References Cited

##### UNITED STATES PATENTS

|           |         |           |
|-----------|---------|-----------|
| 1,458,605 | 6/1923  | Woodward. |
| 2,653,494 | 9/1953  | Creutz    |
| 2,960,763 | 11/1963 | Reichl    |
| 3,122,828 | 3/1964  | Havel     |

#### OTHER REFERENCES

Space Age Materials Extruded by New Techniques, by Paul Lowenstein, in The Tool and Manufacturing Engineering, vol. 50, No. 5, May 1963, pp. 85-91.

JOHN F. CAMPBELL, Primary Examiner.

PAUL M. COHEN, Assistant Examiner.